

# United States Patent Office

3,078,997  
Patented Feb. 26, 1963

1

3,078,997

## FLOTATION PROCESS FOR CONCENTRATION OF PHENACITE AND BERTRANDITE

Richard Havens, Salt Lake City, Utah, assignor to the United States of America as represented by the Secretary of the Interior  
No Drawing. Filed Feb. 24, 1961, Ser. No. 101,616  
15 Claims. (Cl. 209—166)  
(Granted under Title 35, U.S. Code (1952), sec. 266)

The invention herein described and claimed may be manufactured and used by or for the Government of the United States of America for governmental purposes without the payment of royalties thereon or therefor.

This invention relates to the beneficiation of phenacite ( $2\text{BeO}\cdot\text{SiO}_2$ ), bertrandite ( $4\text{BeO}\cdot2\text{SiO}\cdot\text{H}_2\text{O}$ ), and associations thereof with the mineral beryl ( $3\text{BeO}\cdot\text{Al}_2\text{O}_3\cdot6\text{SiO}_2$ ), from their ores.

Recently the discovery of large deposits of low grade ore containing phenacite and bertrandite, sometimes associated with beryl, has raised the possibility of these deposits being a source of beryllium. The ores contain, in addition to the beryllium minerals, quartz, calcite, manganese calcite, fluorite, muscovite, sericite, apatite, and other associated minerals. To be useful, the beryllium minerals must be separated from the mass of gangue material by a simple and inexpensive process.

Accordingly, it is the main object of this invention to provide a simple and economical method for concentrating phenacite, bertrandite, and beryl, if present, from low grade ores, to a degree such that further processing to recover beryllium may be successfully undertaken.

It is an object of the present invention to provide a process for the recovery of larger quantities of phenacite, bertrandite, and beryl from their ores than may be recovered by presently known methods.

A further object of this invention is to provide an improved froth flotation method for the separation, concentration and recovery of phenacite, bertrandite, and beryl from ores, with the production of a material of sufficient beryllium content to be utilized by extractive metallurgical processes.

Yet another object of this invention is to provide an improved froth flotation process for the separation, concentration and recovery of phenacite, bertrandite, and beryl from ores, by the use of water soluble inorganic fluoride and polyphosphates as conditioners.

Other objects and advantages will be apparent from the rest of the disclosure.

In general, the invention comprises separation of phenacite, bertrandite, and beryl from associated minerals, such as quartz, calcite, manganese calcite, fluorite, sericite, apatite, and micas by a flotation process. Many of these minerals, under normal conditions, also tend to respond to fatty acid flotation. To increase the selectivity of the froth flotation process, depressants are added to prevent the entry of undesired minerals into the froth. I have discovered that fluoride ions, and polyphosphate ions, with or without borate ions accomplish this result. Crushed ore in the form of an aqueous pulp is treated with a water soluble fluoride, such as sodium fluoride for example, and a water soluble polyphosphate such as sodium hexametaphosphate (Calgon), or a mixture of Calgon and tetrasodium pyrophosphate, or Calgon and borax.

A small amount of flocculating agent, such as alum or aluminum sulfate, sometimes is useful in flocculating the concentrate or froth for fast removal from the flotation cell. In addition, these agents exert a minor supplemental depressant effect on fluorite and other gangue materials.

After a few minutes conditioning time, a collector oil such as oleic acid, tall oil fatty acid, fish oil fatty acids, etc., is added to the pulp. Kerosine may be added to the

2

collector, if desired. Then, after a short additional conditioning period, air is passed into the pulp, and the froth concentrate recovered.

The residual pulp is reconditioned with Calgon and fatty acid type collector and froth floated again, recovering a second concentrate which may be treated separately or with the first recovered concentrate, or recycled to the first treatment. This process may be repeated with the second tailings, if desired.

10 The process is carried out at room temperature and atmospheric pressure conditions, and the conditioning time periods may vary from 1 to 15 minutes or more. Usually only several minutes are required as a maximum. As depressants, compounds supplying the fluorine ion may be the water soluble inorganic fluorides such as alkali metal fluorides. Ammonium fluoride or hydrogen fluoride may be used on pulps having little calcareous gangue. Sodium fluoride is generally used, however, as it is the most readily available. About 2 to 6 pounds of fluoride per ton of ore is added.

15 Alakli metal polyphosphates are employed as the source of polyphosphate ions, sodium hexametaphosphate (Calgon) being the most readily available source. Mixtures of tetrasodium pyrophosphate and borax may be employed either alone or admixed with Calgon, or borax and Calgon. About 0.5 to 5 pounds per ton of ore of the phosphate conditioner is employed.

20 Collecting agents which may be employed in the process are the fatty acids. These include, for example, oleic acid, fish oil acids, tall oil (which comprises mixtures of rosin acids and fatty acids), linoleic acid, etc. About 1 pound per ton of ore is added. Kerosine may be added to the collecting agent in an amount of from about 0.5 to about 1.0 pound per ton of ore. The kerosine helps depress fluorite and other gangue material, as well as serving as a collector in conjunction with the fatty acid. Other neutral oils such as light or medium fuel oils may be substituted for kerosine. No special frother is required, a fatty acid collector fulfills this function in the instant process under alkaline conditions. Use herein of alkaline metal polyphosphates generally insures this, but if necessary, soda ash or caustic soda may be employed to bring pH to the required value, which may be within the range of from about 7.5 to 9.4.

25 45 Although it is generally necessary to soften the water when using fatty acids as collectors to prevent the formation of insoluble soaps, this is not required in the instant invention. Apparently, the polyphosphate conditioner also serves to prevent the precipitation of insoluble soaps.

50 50 The general method for carrying out the ore treatment according to this invention is as follows:

Crushed ore is wet ground fine enough (passing a 65 mesh screen) to liberate the beryllium-bearing mineral from the gangue minerals. The pulp, a physical mixture of finely ground ore and water, is transferred to a mechanically agitated laboratory flotation cell and then conditioned with 2 to 6 pounds per ton of sodium fluoride and 0.5 to 1 pounds per ton of sodium hexametaphosphate (Calgon), tetrasodium pyrophosphate and borax, Calgon and borax, or mixtures of all three. After a few minute conditioning time, oleic acid, tall oil fatty acid, or similar collector, in an amount of 1 pound per ton of ore, is added to the pulp with or without 0.5 to 1 pound per ton of kerosine per ton of ore, and conditioned for an additional few minutes. The phenacite, bertrandite, and beryl, if present, then are froth floated from the agitated pulp by admitting air to the flotation cell. This product would be designated rougher concentrate No. 1. A second rougher concentrate of lower grade then is froth floated as a separate product by first reconditioning the residual pulp with additional Calgon and fatty acid type collector such as oleic acid, fish oil fatty acids, purified paper mill fat-

70

acids, etc., using about 0.2 to 1 pound Calgon and 0.5 pound of fatty acid per ton of original ore. This product may either be combined with the first rougher concentrate for cleaning or set aside in batch operation. In continuous plant processing, it is recycled through the roughing circuit, and enables mineral recoveries greater than those in the batch tests.

#### EXAMPLE 1

This example illustrates the poor results obtained when the depressants of this invention are not employed.

A typical ore sample containing, in percent, 2 phenacite, 20 calcite, 2 fluorite, 10 sericite, 60 quartz, and 6 other minerals, and assaying 0.73 percent BeO, was wet ground through minus-65-mesh in a laboratory ball mill and froth floated using  $\text{Na}_2\text{SiO}_3$  and  $\text{Na}_2\text{CO}_3$  as conditioning reagents and oleic acid as the collector reagent. The rougher concentrate was cleaned using the same conditioning reagents. The cleaned concentrate assayed 1.68 percent BeO and contained 52 percent of the beryllium in the ore. The rougher tailing from flotation contained 9 percent of the beryllium in the ore and assayed 0.22 percent BeO. Only low recovery of beryllium and a poor degree of upgrading were achieved on this typical phenacite ore by conventional fatty acid flotation.

The following examples give the results obtained with various ore samples and modification of the process.

#### EXAMPLE 2

A phenacite sample from the Mt. Wheeler mine near Ely, Nevada, assayed in percent: 0.72 BeO; 17.1  $\text{CaCO}_3$ ; and 1.9  $\text{CaF}_2$ . Approximate mineral composition of this ore, in percent, was 2 phenacite, 60 quartz, 20 calcite, 2 fluorite, 10 sericite, and 6 other minerals. The sample of ore was wet ground at 50 percent solids in an iron ball mill for 30 minutes to give a product approximately minus-50-mesh. Relatively hard (with reference to dissolved salts) Salt Lake City tap water containing about 200 parts per million total hardness was used throughout the test. The ground pulp was diluted to 30 percent solids with water in a flotation cell and conditioned with sodium fluoride and Calgon; oleic acid then was added as the collector and frother, and the phenacite floated as concentrate 1. The residual pulp was conditioned with Calgon and then with oleic acid, and a second concentrate (concentrate 2) was recovered by floating.

The reagents used, test conditions, and test results are shown in Table 1.

Table 1.—Test Conditions and Flotation Results

#### TEST CONDITIONS

| Treatment or product             | Time of treatment, min. | Reagents, lb./ton of ore |        |            |     |
|----------------------------------|-------------------------|--------------------------|--------|------------|-----|
|                                  |                         | NaF                      | Calgon | Oleic acid | pH  |
| Conditioning.....                | 5                       | 4.0                      | 2.0    | —          | —   |
| Do.....                          | 3                       | —                        | —      | 1.0        | —   |
| Concentrate 1 (by frothing)..... | 1.5                     | —                        | —      | —          | 9.4 |
| Conditioning.....                | 4                       | —                        | —      | 1.0        | —   |
| Do.....                          | 2                       | —                        | —      | .5         | 9.4 |
| Concentrate 2 (by frothing)..... | 3                       | —                        | —      | —          | —   |

#### RESULTS OF FLOTATION

| Product              | Weight, percent | Assay, BeO, percent | Distribution, BeO, percent |
|----------------------|-----------------|---------------------|----------------------------|
| Concentrate 1.....   | 13.7            | 4.8                 | 85.6                       |
| Concentrate 2.....   | 7.6             | .31                 | 3.1                        |
| Rougher tailing..... | 78.7            | .11                 | 11.3                       |
| Calculated head..... | 100.0           | .77                 | 100.0                      |

#### EXAMPLE 3

A composite sample prepared from six ores from various parts of the same mine, assayed, in percent: 0.61 BeO, 0.7  $\text{CaCO}_3$ , 38.3  $\text{SiO}_2$ , 5.0  $\text{CaF}_2$ , and 5.1  $\text{Al}_2\text{O}_3$ . The mineral composition of this sample was, in percent: 1 phenacite, 1 bertrandite, 30 quartz, 27 mangano-calcite,

17 calcite, 4 fluorite, 8 micas, and 12 other minerals. The sample was ball-mill ground for 7 minutes at 50 percent solids to pass a 65-mesh screen and then pulped in a flotation cell to about 30 percent solids. The pulp was conditioned with sodium fluoride, Calgon, and tetrasodium pyrophosphate, then with kerosine and oleic acid. Concentrate was then recovered. Oleic acid was added to the residual pulp and a second concentrate (concentrate 2) then was froth floated. The kerosine helped to depress the fluorite and, with the oleic acid, to collect the beryllium minerals. The reagents used, test conditions, and results are given in Table 2.

Table 2.—Test Conditions and Flotation Results

| Treatment or product             | Time of treatment, min. | TEST CONDITIONS |        |                   |            |          |
|----------------------------------|-------------------------|-----------------|--------|-------------------|------------|----------|
|                                  |                         | NaF             | Calgon | TSPP <sup>1</sup> | Oleic acid | Kerosine |
| Conditioning.....                | 2.9                     | 4.0             | 3.0    | 1.0               | —          | —        |
| Do.....                          | 2.6                     | —               | —      | —                 | 0.52       | 0.53     |
| Concentrate 1 (by frothing)..... | 1                       | —               | —      | —                 | —          | —        |
| Conditioning.....                | 3                       | —               | —      | —                 | .80        | —        |
| Concentrate 2 (by frothing)..... | 1                       | —               | —      | —                 | —          | —        |

#### RESULTS OF FLOTATION

| Product              | Weight, percent | Assay, BeO, percent | Distribution, BeO, percent |
|----------------------|-----------------|---------------------|----------------------------|
| Concentrate 1.....   | 3.0             | 15.0                | 68.5                       |
| Concentrate 2.....   | 4.1             | 2.1                 | 13.1                       |
| Rougher tailing..... | 92.9            | .13                 | 18.4                       |
| Calculated head..... | 100.0           | .66                 | 100.0                      |

<sup>1</sup> Tetrasodium pyrophosphate.

<sup>2</sup> 3 min. after each reagent addition.

#### EXAMPLE 4

This example demonstrates that adjustments in the basic test conditions and reagent schedules may be made to achieve even better results than illustrated by Example 3.

The same composite ore was wet ground and pulped as in Example 3, and then froth floated in the manner there shown, using the specific test conditions listed in Table 3, with the results as tabulated.

Table 3.—Test Conditions and Flotation Results

| Treatment or product             | Time of treatment, min. | TEST CONDITIONS |        |                   |            |          |
|----------------------------------|-------------------------|-----------------|--------|-------------------|------------|----------|
|                                  |                         | NaF             | Calgon | TSPP <sup>1</sup> | Oleic acid | Kerosine |
| Conditioning.....                | 2.9                     | 4.0             | 2.5    | 0.8               | —          | —        |
| Do.....                          | 2.3                     | —               | —      | —                 | 1.05       | 0.53     |
| Concentrate 1 (by frothing)..... | 1.5                     | —               | —      | —                 | —          | —        |
| Conditioning.....                | 1.5                     | —               | —      | —                 | .35        | —        |
| Concentrate 2 (by frothing)..... | 1.5                     | —               | —      | —                 | —          | —        |

#### RESULTS OF FLOTATION

| Product              | Weight, percent | Assay, BeO, percent | Distribution, BeO, percent |
|----------------------|-----------------|---------------------|----------------------------|
| Concentrate 1.....   | 2.4             | 18.1                | 68.5                       |
| Concentrate 2.....   | 2.5             | 4.6                 | 16.5                       |
| Rougher tailing..... | 95.1            | 0.10                | 15.0                       |
| Calculated head..... | 100.0           | 0.63                | 100.0                      |

<sup>1</sup> Tetrasodium pyrophosphate.

<sup>2</sup> 3 min. after each reagent addition.

<sup>3</sup> 1.5 min. after each reagent addition.

## 5 EXAMPLE 5

This sample, from the same deposit, was a composite of two ores. In percent its assay was 0.49 BeO, 30.8 CaCO<sub>3</sub>, 16.2 CaF, 4.8 Al<sub>2</sub>O<sub>3</sub>, 2.7 Fe, and 0.17 WO<sub>3</sub>. The mineral composition of this ore, in percent, was 0.4 phenacite, 0.9 bertrandite, 26 manganocalcite, 15 calcite, 17 quartz, 14 micas, 7 feldspar, 17 fluorite, and 2.7 other minerals. The flotation sample was wet ground at 50 percent solids in a ball mill to approximately minus-65-mesh and pulped at 30 percent solids in a flotation cell. The steps of conditioning and recovery were similar to those described in Example 2.

The reagents test conditions, and test results are given in Table 4.

*Table 4.—Test Conditions and Flotation Results*

| Treatment or product        |  | Time of treatment, min. | Reagents, lb./ton of ore |        |       |            |          |
|-----------------------------|--|-------------------------|--------------------------|--------|-------|------------|----------|
|                             |  |                         | NaF                      | Calgon | Borax | Oleic acid | Kerosene |
| Conditioning                |  | 1.9                     | 4.0                      | 3.0    | 0.1   | 1.05       | 0.53     |
| Do                          |  | 1.3                     |                          |        |       |            |          |
| Concentrate 1 (by frothing) |  | 1.5                     |                          |        |       |            |          |
| Conditioning                |  | 1.0                     |                          |        | .1    |            |          |
| Do                          |  | 1.5                     |                          |        |       | .35        | .27      |
| Concentrate 2 (by frothing) |  | 1.5                     |                          |        |       |            |          |

### RESULTS OF FLOTATION

| Product         | Weight, percent | Assay, BeO, percent | Distribution, BeO, percent |
|-----------------|-----------------|---------------------|----------------------------|
| Concentrate 1   | 3.4             | 10.9                | 66.7                       |
| Concentrate 2   | 1.6             | 3.85                | 11.1                       |
| Rougher tailing | 95.0            | .13                 | 22.2                       |
| Calculated head | 100.0           | .55                 | 100.0                      |

<sup>1</sup> 3 min. after each reagent addition.

<sup>2</sup> 1.5 min. after each reagent addition.

## EXAMPLE 6

A second ore sample from Mt Wheeler mine near Ely, Nev., assayed, in percent, 4.7 BeO, 4.3 CaCO<sub>3</sub>, 3.0 CaF<sub>2</sub>, 60.7 SiO<sub>2</sub>, and 4.2 Fe. The approximate mineral composition of this ore, in percent, was 10 phenacite, 3 fluorite, 4.5 calcite, with the balance comprised of micas, quartz, feldspars, sulfides, and limonite. The sample of ore was ground in the presence of NaF and a sulfide collector, such as the xanthates or thiophosphates for example, for 7 minutes at 50 percent solids to approximately minus-65-mesh. It then was pulped in a flotation cell to about 30 percent solids and conditioned with Calgon and a frother, e.g. pine oil or a cresol, etc. The sulfides were then removed by froth flotation as a sulfide concentrate. The pulp remaining in the flotation cell then was conditioned with oleic acid and fuel oil and a phenacite concentrate froth floated to form a concentrate 1. A second and third concentrate (concentrates 2 and 3) also were floated with additional oleic acid and fuel oil. The three rougher concentrates 1, 2 and 3 were combined and conditioned with additional Calgon, oleic acid and fuel oil and froth floated to recover a cleaner concentrate. Additional Calgon was added thereto and a recleaned concentrate I was recovered. The residual pulp was conditioned with additional oleic acid and fuel oil and a concentrate II was recovered by frothing.

50

55

65

70

## 6

The reagents used, test conditions, and results are summarized in Table 5.

*Table 5.—Test Conditions and Flotation Results*

### TEST CONDITIONS

| Treatment or product              | Time of treatment, min. | Reagents, lb./ton of ore |                  |          |        |            |          |
|-----------------------------------|-------------------------|--------------------------|------------------|----------|--------|------------|----------|
|                                   |                         | NaF                      | Z-6 <sup>1</sup> | Pine oil | Calgon | Oleic acid | Fuel oil |
| Grind                             | 7                       | 4.0                      | 0.1              |          |        |            |          |
| Conditioning                      |                         |                          |                  | 0.04     | 0.75   |            |          |
| Sulfide concentrate (by frothing) | 5                       |                          |                  |          |        |            |          |
| Conditioning                      | 2                       |                          |                  |          |        | 1.75       | 0.7      |
| Concentrate 1 (by frothing)       | 5                       |                          |                  |          |        |            |          |
| Conditioning                      | 2                       |                          |                  |          |        | .9         | .35      |
| Concentrate 2 (by frothing)       | 5                       |                          |                  |          |        |            |          |
| Conditioning                      | 2                       |                          |                  |          |        | .9         | .35      |
| Concentrate 3 (by frothing)       | 3                       |                          |                  |          |        |            |          |
| Cleaner conditioning              | 3                       |                          |                  |          |        | .1         | .25      |
| Cleaner concentrate (by frothing) | 5                       |                          |                  |          |        |            |          |
| Recleaner conditioning            | 3                       |                          |                  |          | .1     |            |          |
| Concentrate I (by frothing)       | 4                       |                          |                  |          |        |            |          |
| Conditioning                      | 3                       |                          |                  |          |        | .25        | .70      |
| Concentrate II (by frothing)      | 2                       |                          |                  |          |        |            |          |

<sup>1</sup> Z-6 is the trade name for a collecting agent consisting of mixed amyl xanthates.

35

### RESULTS OF FLOTATION

| Product                       | Weight, percent | Assay, BeO, percent | Distribution, BeO, percent |
|-------------------------------|-----------------|---------------------|----------------------------|
| Sulfide concentrate           | 0.4             | 2.4                 | 0.2                        |
| Concentrate I                 | 8.9             | 35.2                | 68.1                       |
| Concentrate II                | 2.9             | 26.5                | 16.5                       |
| Cleaner and recleaner tailing | 8.5             | 4.4                 | 8.1                        |
| Rougher tailing               | 79.3            | .4                  | 7.1                        |
| Calculated head               | 100.0           | 4.6                 | 100.0                      |

## EXAMPLE 7

A sample of ore from the Badger flats area in Colorado, assayed in percent, 0.5 BeO, 0.13 Li<sub>2</sub>O, 72.9 SiO<sub>2</sub>, 3.6 Fe, and 13.0 Al<sub>2</sub>O<sub>3</sub>. The mineral composition of this ore in percent was: 1 bertrandite, 0.3 beryl, 0.1 euclase, 40 quartz, 33 micas, 20 feldspar, with minor amounts of limonite, hematite, fluorite, calcite, lead and zinc carbonates, and sulfide minerals. A sample of the ore was treated under the conditions and with reagents shown in Table 6. The ore was ground in the presence of NaF for 12 minutes at 50 percent solids in a laboratory ball mill to approximately 100-mesh and pulped in a flotation cell. It then was conditioned by adding Calgon and floated to form rougher concentrate 1. The residual pulp was conditioned by adding oleic acid and kerosene thereto, and a second concentrate (rougher concentrate 2) was floated. The two rougher concentrates were combined, conditioned with Calgon and then with oleic acid, kerosine and borax, and floated to recover concentrate I.

The reagents test conditions, and results of flotation are given in Table 6.

Recycling of the cleaner tailing in a continuous plant would improve over-all beryllium recovery.

Table 6.—Test Conditions and Flotation Results  
TEST CONDITIONS

| Treatment or product                   | Time of treatment min. | Reagents, lb./ton of ore |         |            |           |       |      |
|----------------------------------------|------------------------|--------------------------|---------|------------|-----------|-------|------|
|                                        |                        | NaF                      | Cal-gon | Oleic acid | Kero-sine | Borax | pH   |
| Grind                                  | 12                     | 3.0                      |         |            |           |       |      |
| Conditioning                           | 5                      |                          | 0.75    |            |           |       |      |
| Do                                     | 2                      |                          |         | 1.0        | 0.5       |       | 8.2  |
| Rougher concentrate 1<br>(by frothing) | 3                      |                          |         |            |           |       |      |
| Conditioning                           | 2                      |                          |         |            | .5        | .25   | 0.05 |
| Rougher concentrate 2<br>(by frothing) | 2                      |                          |         |            |           |       |      |
| Cleaner conditioning                   | 3                      |                          |         | .5         |           |       |      |
| Do                                     | 3                      |                          |         |            | .5        | .25   | .05  |
| Concentrate I (by frothing)            | 3                      |                          |         |            |           |       |      |

## RESULTS OF FLOTATION

| Product             | Weight, percent | Assay, BeO, percent | Distribution, BeO, percent |
|---------------------|-----------------|---------------------|----------------------------|
| Cleaner concentrate | 2.63            | 12.2                | 59.9                       |
| Cleaner tailing     | 5.09            | 1.64                | 15.6                       |
| Rougher tailing     | 92.28           | .14                 | 24.5                       |
| Calculated head     | 100.0           | 0.53                | 100.0                      |

It will be appreciated from a study of the foregoing specification that the invention described therein is capable of various modifications and changes without departing from its essential spirit and scope.

I claim:

1. A process for the concentration of a beryllium mineral selected from the class consisting of phenacite, bertrandite, beryl, and mixtures thereof from an ore containing the same together with a sulfide mineral and gangue, which comprises: forming an aqueous pulp of said ore, removing the sulfide mineral therefrom by adding to the pulp a sulfide collector and a frother, frothing the said pulp to remove the sulfide mineral as a froth and leaving a residual pulp containing the beryllium minerals, adding to the residual pulp (1) a depressant for the gangue comprising a water soluble inorganic fluoride and an alkali metal inorganic polyphosphate; maintaining the pH of the resulting pulp at a range of from about 7.5 to about 9.4; (2) a fatty acid type collector for the beryllium mineral comprising a member of the class consisting of higher fatty acids, and a light neutral hydrocarbon oil together with a higher fatty acid; and then froth floating the beryllium minerals from the gangue.

2. A process for the concentration of a beryllium mineral selected from the class consisting of phenacite, bertrandite, beryl, and mixtures thereof from an ore containing the same together with gangue, which comprises: adding to an aqueous pulp of said ore (1) a depressant for the gangue comprising a water soluble inorganic fluoride and an alkali metal inorganic polyphosphate; (2) a fatty acid type collector for the beryllium mineral comprising a member of the class consisting of higher fatty acid, and a light neutral hydrocarbon oil together with a higher fatty acid; (3) a flocculant comprising aluminum sulfate; maintaining the pH of the resulting pulp at a range of from about 7.5 to about 9.4; and then froth floating the beryllium minerals from the gangue.

3. A process for the concentration of a beryllium mineral selected from the class consisting of phenacite, bertrandite, beryl, and mixtures thereof from an ore containing the same, together with gangue, which comprises: adding to an aqueous pulp of said ore (1) a depressant for the gangue comprising an alkali metal fluoride and an alkali metal polyphosphate; (2) a fatty acid type collector for the beryllium mineral comprising a member of the class consisting of higher fatty acid, and

a light neutral hydrocarbon oil together with a higher fatty acid; maintaining the pH of the resulting pulp at a range of from about 7.5 to about 9.4; and then froth floating the beryllium minerals from the gangue.

4. A process for the concentration of a beryllium mineral selected from the class consisting of phenacite, bertrandite, beryl, and mixtures thereof from an ore containing the same, together with gangue, which comprises: adding to an aqueous pulp of said ore (1) a depressant for the gangue comprising sodium fluoride and sodium hexametaphosphate; (2) a fatty acid type collector for the beryllium mineral comprising a member of the class consisting of higher fatty acid, and a light neutral hydrocarbon oil together with a higher fatty acid; maintaining the pH of the resulting pulp at a range of from about 7.5 to about 9.4; and then froth floating the beryllium minerals from the gangue.

5. A process for the concentration of a beryllium mineral selected from the class consisting of phenacite, bertrandite, beryl, and mixtures thereof from an ore containing the same, together with gangue, which comprises: adding to an aqueous pulp of said ore (1) a depressant for the gangue comprising sodium fluoride and sodium hexametaphosphate; (2) a fatty acid type collector for the beryllium mineral comprising a member of the class consisting of higher fatty acid, and a light neutral hydrocarbon oil together with a higher fatty acid; (3) a flocculant comprising aluminum sulfate; maintaining the pH of the resulting pulp at a range of from about 7.5 to about 9.4; and then froth floating the beryllium minerals from the gangue.

6. A process for the concentration of a beryllium mineral selected from the class consisting of phenacite, bertrandite, beryl, and mixtures thereof from an ore containing the same together with gangue, which comprises: adding to a pulp of said ore (1) a depressant for the gangue comprising sodium fluoride and sodium hexametaphosphate; (2) a collector for the beryllium mineral consisting of a higher fatty acid and kerosine; maintaining the pH of the resulting pulp at a range of from about 7.5 to about 9.4; and then froth floating the beryllium minerals from the gangue.

7. A process for the concentration of a beryllium mineral selected from the class consisting of phenacite, bertrandite, beryl, and mixtures thereof from an ore containing the same, together with gangue, which comprises: adding to an aqueous pulp of said ore (1) a depressant for the gangue comprising sodium fluoride, sodium hexametaphosphate and tetrasodium pyrophosphate; (2) a fatty acid type collector for the beryllium mineral comprising a member of the class consisting of higher fatty acid, and a light neutral hydrocarbon oil together with a higher fatty acid; maintaining the pH of the resulting pulp at a range of from 7.5 to about 9.4; and then froth floating the beryllium minerals from the gangue.

8. A process for the concentration of beryllium mineral selected from the class consisting of phenacite, bertrandite, beryl, and mixtures thereof from an ore containing the same, together with gangue, which comprises: adding to an aqueous pulp of said ore (1) a depressant for the gangue comprising sodium fluoride, sodium hexametaphosphate and borax; (2) a fatty acid type collector for the beryllium mineral comprising a member of the class consisting of higher fatty acid, and a light neutral hydrocarbon oil together with a higher fatty acid; maintaining the pH of the resulting pulp at a range of from about 7.5 to about 9.4; and then froth floating the beryllium mineral from the gangue.

9. A process for the concentration of a beryllium mineral selected from the class consisting of phenacite, bertrandite, beryl, and mixtures thereof from an ore containing the same together with gangue, which comprises: adding to an aqueous pulp of said ore (1) a depressant for the gangue comprising a water soluble inorganic fluoride and an alkali metal inorganic polyphosphate;

(2) a fatty acid type collector for the beryllium mineral comprising a member of the class consisting of a higher fatty acid, and a light neutral hydrocarbon oil together with a higher fatty acid; maintaining the resulting pulp at a pH in the range of from about 7.5 to about 9.4; froth floating a first concentrate of the beryllium mineral from the gangue; separating the said first concentrate and gangue; reconditioning the tailings by adding to an aqueous pulp thereof (3) a gangue depressant selected from the class consisting of alkali metal inorganic polyphosphate borax and mixtures thereof, as required; and (4) a fatty acid type collector of the class consisting of higher fatty acids, and a light neutral hydrocarbon oil together with a fatty acid; maintaining the pH of the tailings pulp at a range of from about 7.5 to about 9.4; and then froth floating a second concentrate of beryllium minerals from the said tailings.

10. The method of claim 9 wherein an aluminum sulfate flocculant is added to aqueous ore pulp together with conditioners and depressants.

11. The method of claim 9 wherein the second beryllium mineral concentrate is recycled to the aqueous ore pulp in the first froth floating step.

12. A process for the concentration of a beryllium mineral selected from the class consisting of phenacite, bertrandite, beryl, and mixtures thereof from an ore containing the same together with gangue, which comprises: adding to an aqueous pulp of said ore a depressant for the gangue consisting of 2 to 6 pounds of sodium fluoride per ton of ore, 0.5 to 5 pounds per ton of ore of a member of the class consisting of sodium hexametaphosphate, tetrasodium pyrophosphate, borax and mixtures thereof, the borax always being admixed with at least one of the other members of the class; a collector for the beryllium mineral comprising a member of the class consisting of a higher fatty acid, and a light neutral hydrocarbon oil together with a higher fatty acid, the higher fatty acid being in an amount of about 1 pound

per ton of ore and the said hydrocarbon oil in an amount of from about 0.5 to about 1 pound per ton of ore; and froth floating the beryllium minerals from the gangue.

13. The method of claim 12, wherein the gangue depressant consists of about 4 pounds of sodium fluoride, and about 2 pounds of sodium hexametaphosphate, and the collector consists of about 1.0 pound of oleic acid, all the weights being in pounds per ton of ore.

14. The method of claim 12, wherein the gangue depressant consists of about 4.0 pounds of sodium fluoride, about 3 pounds of sodium hexametaphosphate, about 1.0 pound of tetrasodium pyrophosphate, and the collector consists of about 0.5 pound of oleic acid and 0.5 pound of kerosine, all of the weights being in pounds per ton of ore.

15. The method of claim 12, wherein the gangue depressant consists of about 4.0 pounds sodium fluoride, 3.0 pounds sodium hexametaphosphate, 0.1 pound borax, and the collector consists of about 1.0 pounds of oleic acid and about 0.5 pound of kerosine, all of the weights being in pounds per ton of ore.

#### References Cited in the file of this patent

##### UNITED STATES PATENTS

|           |         |       |               |
|-----------|---------|-------|---------------|
| 2,040,187 | Rose    | ----- | May 12, 1936  |
| 2,373,305 | Gieseke | ----- | Oct. 7, 1942  |
| 2,385,819 | Lamb    | ----- | Oct. 2, 1945  |
| 2,424,552 | Clemmer | ----- | July 29, 1947 |
| 2,666,587 | Runke   | ----- | Jan. 19, 1954 |
| 2,797,808 | Tueter  | ----- | July 2, 1957  |

##### OTHER REFERENCES

United States Bureau of Mines RI 4040, March 1947.

35 Eigles et al.: Floatability of Beryl, Second U. N. International Conference on the Peaceful Uses of Atomic Energy, volume 3, 1958, pages 162-166.